



US006319604B1

(12) **United States Patent**  
**Xu**

(10) **Patent No.:** **US 6,319,604 B1**  
(45) **Date of Patent:** **Nov. 20, 2001**

(54) **ABRASION RESISTANT COATED WIRE**(75) Inventor: **James J. Xu**, Fort Wayne, IN (US)(73) Assignee: **Phelps Dodge Industries, Inc.**, Fort Wayne, IN (US)

( \*) Notice: Subject to any disclaimer, the term of this patent is extended or adjusted under 35 U.S.C. 154(b) by 0 days.

(21) Appl. No.: **09/436,272**(22) Filed: **Nov. 8, 1999****Related U.S. Application Data**

(60) Provisional application No. 60/142,842, filed on Jul. 8, 1999, now abandoned.

(51) **Int. Cl.<sup>7</sup>** ..... **B32B 15/00**; H01B 7/00(52) **U.S. Cl.** ..... **428/379**; 428/372; 428/383; 428/389; 174/110 SR; 174/102 P; 174/110 FC; 174/110 PM; 174/110 N(58) **Field of Search** ..... 428/372, 379, 428/383, 389; 174/110 SR, 110 N, 110 PM, 110 FC, 120 SR, 102 P(56) **References Cited**

## U.S. PATENT DOCUMENTS

|           |         |                     |
|-----------|---------|---------------------|
| 3,615,913 | 10/1971 | Shaw .              |
| 4,340,697 | 7/1982  | Aya et al. .        |
| 4,342,814 | 8/1982  | Usuki et al. .      |
| 4,350,738 | 9/1982  | Saunders et al. .   |
| 4,377,652 | 3/1983  | Ohmura et al. .     |
| 4,405,687 | 9/1983  | Morita et al. .     |
| 4,426,423 | 1/1984  | Intrater et al. .   |
| 4,476,192 | 10/1984 | Imai et al. .       |
| 4,503,124 | 3/1985  | Keane et al. .      |
| 4,563,369 | 1/1986  | Lavallee .          |
| 4,693,936 | 9/1987  | McGregor et al. .   |
| 4,716,079 | 12/1987 | Sano et al. .       |
| 4,935,302 | 6/1990  | Hjortsberg et al. . |
| 5,066,513 | 11/1991 | Zurecki et al. .    |
| 5,209,987 | 5/1993  | Penneck et al. .    |

|             |        |                            |
|-------------|--------|----------------------------|
| 5,296,260   | 3/1994 | Sawada et al. .            |
| 5,350,638   | 9/1994 | Sawada et al. .            |
| 5,393,612   | 2/1995 | Matsuura et al. .          |
| 5,425,992   | 6/1995 | Tachikawa et al. .         |
| 5,443,905   | 8/1995 | Sawada et al. .            |
| 5,861,578   | 1/1999 | Hake et al. .              |
| 5,902,681 * | 5/1999 | Ueoka et al. ..... 428/383 |

## FOREIGN PATENT DOCUMENTS

|             |   |                |
|-------------|---|----------------|
| 54-99137    | * | 4/1979 (JP) .  |
| 63-81173    |   | 4/1988 (JP) .  |
| 3-245417    |   | 11/1991 (JP) . |
| 5-320340    |   | 12/1993 (JP) . |
| 09294652    |   | 10/1997 (JP) . |
| WO 86/03329 |   | 6/1986 (WO) .  |

## OTHER PUBLICATIONS

Brochure—Poly-Thermaleze®TW (PTZ TW), Phelps Dodge Magnet Wire Company 1998.

Article—*Improved Tough Wire*, James J. Xu, Phelps Dodge Magnet Wire Company, undated.Article—*Dynamic Mechanical Properties of Tough Magnet Wire*, James J. Xu et al., Phelps Dodge Magnet Wire Company, Oct. 1998.Article—*Synthesis and characterization of a rubber incorporated polyamideimide*, Debasish Sen et al, *Makromol. Chem.*, 186, 1625–1630 (1985).

\* cited by examiner

Primary Examiner—Cynthia H. Kelly

Assistant Examiner—J. M. Gray

(74) Attorney, Agent, or Firm—Barnes &amp; Thornburg

(57) **ABSTRACT**

A coated wire that includes an electrical conductor having an abrasion and varnish craze resistant lubricated coating. The coating is made of a ceramic particulate material dispersed in a polyamideimide binder. Ceramic particulate materials suitable for incorporation in the coatings include silicon nitride ( $Si_3N_4$ ), aluminum nitride (AlN), and titanium nitride (TiN).

17 Claims, 2 Drawing Sheets





FIG. 1



FIG. 2



FIG. 3



FIG. 4

## ABRASION RESISTANT COATED WIRE

## RELATED APPLICATIONS

The present application is based upon U.S. Provisional Application Ser. No. 60/142,842, filed on Jul. 8, 1999, abandoned, the complete disclosure of which is hereby expressly incorporated by reference.

## TECHNICAL FIELD

This invention relates to an electrical conductor having an insulation coating. More particularly, the present invention relates to an electrical conductor having an abrasion and varnish craze resistant lubricated coat system.

## BACKGROUND ART

Coated electrical conductors may comprise one or more electrical insulation layers formed around a conductive core. Magnet wire is one form of coated electrical conductor in which the conductive core is a copper wire, and the insulation layer or layers comprise dielectric materials, such as polymeric resins. Magnet wire is used in the electromagnet windings of transformers, electric motors, and the like. Because of its use in such windings, friction, and abrading forces are often encountered. As a result, this insulation layer can be susceptible to damage.

High voltage-surge failure rate, for example, has been of concern to motor manufacturers. Surge failure is associated with insulation damage resulting from modern, fast automatic winding and abusive coil insertion processes for motor stators. Coating a polyester insulated wire with an abrasion resistant polyamideimide and wax is one way to minimize friction thereby reducing wire surface damage during the winding process. Wires manufactured in this manner, however, can experience surge failure rates of at least about 10,000–20,000 parts per million. Another form of failure is varnish craze. Varnish craze is a small fissure (about 1–2 microns deep) on the surface of the coating. Typically, varnish craze includes several fissures in a localized area that impair the insulative properties of the wire. Therefore, a need exists for a wire coating that will offer high resistance to the various damaging effects to wire coatings, including abrasion, and varnish craze.

## SUMMARY OF THE INVENTION

According to certain features, characteristics, embodiments and alternatives of the present invention which will become apparent as the description thereof proceeds below, the present invention provides an electrical conductor having an abrasion and varnish craze resistant lubricated coat system. The coating is made of a ceramic particulate material dispersed in a polyamideimide binder. Ceramic particulate materials suitable for incorporation in the coatings include silicon nitride ( $Si_3N_4$ ), aluminum nitride (AlN), and titanium nitride (TiN). The particulate size for these ceramic materials generally ranges from 1 to 10 microns. The amount of ceramic particulate material that is used is generally from 1 to 15 percent by weight.

In another embodiment, the coating includes a ceramic particulate material and a fluoroplastic dispersed in a polyamideimide. The ceramic particulate materials being used are the same as those listed above. The fluoroplastics that may be used include polytetrafluoroethylene, polychlorotrifluoroethylene, polyvinylidene fluoride, and fluorinated ethylene propylene.

In still another embodiment, the coating includes a ceramic particulate material with polyethylene dispersed in

polyamideimide. The ceramic particulate materials that can be used are, again, the same as those listed above.

In a further embodiment, a base insulation coat may be applied to a conductor. The base insulation coat may be made from any of a variety of heat resistant, electrical insulation materials such as polyetherimide, polyimide, polyesterimide, epoxy resin, polyester used as basecoat and bondable coat, polyarylsulfone, and polyether ether ketone. All of the above embodiments may be used as an enamel topcoat over the insulation coat.

## BRIEF DESCRIPTION OF DRAWINGS

The present invention will be described hereafter with reference to the attached figures which are given as non-limiting examples only, in which:

FIG. 1 is a cross sectional view of an abrasion resistant coated wire according to one embodiment of the present invention;

FIG. 2 is a perspective view of the wire of FIG. 1;

FIG. 3 is a cross sectional view of another embodiment of an abrasion resistant coated wire; and

FIG. 4 is a perspective view of the wire of FIG. 3.

Corresponding reference characters indicate corresponding parts throughout the several figures. The exemplification set out herein.

## DETAILED DESCRIPTION OF THE DRAWINGS

This invention relates to an electrical conductor having an insulation coating. More particularly, the present invention relates to an electrical conductor having an abrasion and varnish craze resistant lubricated coat system. The abrasion resistant coated magnet wire 1 according to one embodiment of the present invention is shown in FIGS. 1 and 2. Magnet wire 1 comprises a coating 3 formed around a conductive core 2. Conductive core 2 is illustratively a copper wire. It is appreciated, however, that core 2 may be formed from any suitable ductile conductive material. For example, core 2 may be formed from copper clad aluminum, silver plated copper, nickel plated copper, aluminum alloy 1350, combinations of these materials, or the like.

Coating 3 may be formed from a ceramic, generally global-shaped particulate material, dispersed in a polyamideimide binder having electrically insulative, flexible properties. Because of its electrically insulative properties, coating 3 helps insulate conductive core 2 as it carries electrical current during motor operations. Because of its flexibility characteristics, coating 3 is resistant to cracking and/or delaminating, as well as being impact and scrape resistant. This substantially improves the wire's toughness so that when it is wound into the windings of an electric motor it will not be damaged.

Coating 3 may be applied peripherally about conductive core 2 by a variety of means. For example, coating 3 may be formed from a prefabricated film that is wound around the conductor. Coating 3 may also be applied using extrusion coating techniques. Alternatively, coating 3 may be formed from one or more fluid thermoplastic or thermosetting polymeric resins and applied to conductor 2, and dried and/or cured using one or more suitable curing and/or drying techniques such as chemical, radiation, or thermal treatments. A variety of such-polymeric resins known to those skilled in the art may be used, including terephthalic acid alkyls, polyesters, polyesterimides, polyetheramides, polyetheramideimides, polyesterurethanes, polyurethanes, epoxy resins, polyamide, polyimides, polyamideimides,

polysulphones, silicone resins, polymers incorporating polyhydantion, phenolic resins, vinyl copolymers, polyolefins, polycarbonates, polyethers, polyetherimides, polyetheramides, polyetheramideimides, polyisocyanates, combinations of these materials, and the like.

Ceramic particulates such as silicon nitride, aluminum nitride and titanium nitride can increase the toughness of wire 1. The amount of ceramic particulates added to coating 3 should be about 1%–15% by weight of the coat with about 3%–6% by weight of the coat preferable. This is because between 3%–6%, the ceramic provides substantial protection yet the wire is still flexible enough to wind properly. If more than 15% by weight ceramic particulate material is added the conductor becomes less flexible, thereby reducing its ability to serve as a magnet wire. In addition, the ceramic material's particle size can be about 1 to 10 microns, preferably 3 to 5 microns. In one embodiment, coating 3 comprises a ceramic particulate material in combination with a fluoropolymer dispersed in a polyamideimide binder. Fluoropolymers that may be used include polytetrafluoroethylene, polychlorotrifluoroethylene, polyvinylidene fluoride and fluorinated ethylene propylene. About 1% of fluoropolymer by weight of coating may be used. In addition, the fluoropolymer may have a particle size ranging from 0.5 to 10 microns. The preferred particle size is 1 to 3 microns creating improved enamel solution stability as well as improved penetration of the particles within the thin film.

In another embodiment, coating 3 comprises a ceramic particulate material in combination with a polyethylene dispersed in a polyamideimide binder. About 1% of polyethylene by weight of coating is used. In addition, the polyethylene may have a particle size ranging from 5 to 15 microns. The preferred particle size may be less than 10 microns for the same reasons previously discussed.

In a still further embodiment, the present invention comprises a dual-layer conductive wire 4 as shown in FIGS. 3 and 4. A topcoat 6 provides additional operational stability for insulation layer 5. Insulation layer 5 is applied peripherally about the electrical conductor 2. Insulation layer 5 may be formed from any insulative material known to those skilled in the art suitable for forming electrically insulative, flexible base coatings for electrical conductors. For example, polyetherimide, polyimide, polyesterimide, epoxy resin, polyester used as basecoat and bondable coat, polyarylsulfone, and polyether ether ketone may be used.

Ceramic-polyamideimide topcoat 6 is then applied peripherally about insulation coat 5. The several embodiments of the ceramic-polyamideimide coating previously discussed may serve as topcoat 6. In addition, ceramic-polyamideimide topcoat 6 comprising either a fluoropolymer or polyethylene as previously discussed may also be used.

The present invention will now be described with respect to the following examples which are intended to be only representative of the manner in which the principles of the present invention may be implemented in actual embodiments. The following examples are not intended to be an exhaustive representation of the present invention. Nor are the following examples intended to limit the present invention only to the precise forms which are exemplified.

#### WORKING EXAMPLES AND COMPARISON TESTS

The following working examples were based on three 18 gauge control wires having different enamel compositions

applied to each wire. For example, control wire I comprised a polyamideimide enamel; control wire II comprised a polyamideimide enamel with polytetrafluoroethylene; and control wire III comprised a polyamideimide enamel with polyethylene. Ceramic nitride particulates were added in varying percentages (by weight) to the enamel composition of each control wire. These test wires were tested via the repeated scrape test and subjected to a coefficient of friction analysis and compared to their respective control wire.

The repeated scrape test is a widely recognized and employed measure of abrasion resistance for wire coatings. The repeated scrape test consists of a test wire suspended adjacent a pendulum having a needle attached at the end thereof. The needle swings back and forth scraping the coating on the periphery of the wire. A defined loading is applied to the pendulum providing a controlled force to the needle against the wire. For the working examples described herein, the control and test wires were tested under a 700-gram load pendulum scraper for an 18 gauge (1 mm diameter) copper wire. The number of strokes (Rptd. S.) it took the scraper to wear through the coatings was recorded. A greater number of strokes before failure indicated a more abrasion resistant coating.

In addition, a dynamic coefficient of friction test was performed on the wires. This test included subjecting the wires under a load of 1000 grams, an 18 AWG wire pulled at a constant speed. The dynamic coefficient of friction (C. of F.) was recorded over approximately 1000 sampling points. A low coefficient of friction indicated a self-lubricating property in the magnet wire enamel reducing the wear on the wire.

The following is the procedure for making control wires I, II and III.

#### Control Wire I

1 mole of Diphenylmethane 4,4'-diisocyanate (MDI), 0.7–1.0 mole of Trimellitic Anhydride (TMA), 0–0.5 mole of Adipic Acid (AA), and 0–0.5 mole of Isophthalic Acid (IPA) were added into mixed solvents of N-Methyl pyrrolidone (NMP) and aromatic solvent NJ100. The reaction was carried out at 70° C.–90° C. for at least three hours and then at 120° C.–150° C. until all the diisocyanate groups disappeared as indicated by a Fourier Transform Infrared spectrometer (FTIR). A small amount of additives such as versar wax, aliphatic diisocyanate, and fluorocarbon-based surfactant may be present. The reaction was then stopped with mixed solvents of alcohol, NMP and NJ100. The solids content was controlled within 26%–30%, and the resultant enamel had a viscosity of 1700–2400 cps at 37.8° C.

The resultant enamel was applied to an 18 AWG copper wire which was precoated with eight passes of polyester basecoat at the speed of 28–60 meters per minute in an oven having temperatures of 450° C.–600° C. The insulation build is approximately 3.0–3.3 mil.

#### Control Wire II

The wire made for control II was made identical to that made for control I but for the addition of 3% (solids/solids) polytetrafluoroethylene powder into the polyamideimide enamel. The typical size of the polytetrafluoroethylene powder was in the range of 1–3 microns. The melting point of polytetrafluoroethylene powder used in this control was approximately 320° C.–340° C.

#### Control Wire III

The wire made for control III was made identical to that made for control I as well, but for the addition of 3% (solids/solids) polyethylene powder into the polyamideimide enamel. The typical size of polyethylene powder was in the range of 1–10 microns. The melting point of polyethylene powder used in this control was approximately 100° C.

Silicon Nitride ( $\text{Si}_3\text{N}_4$ ) Working Examples

Varying amounts of  $\text{Si}_3\text{N}_4$  including 1%, 2%, 3%, 4%, 6%, 9%, 12% and 15% by weight were added to each control wire. Each control wire with  $\text{Si}_3\text{N}_4$  was then tested and compared to each control wire with no  $\text{Si}_3\text{N}_4$  to determine effects on abrasion resistance. The following illustratively describes how the varying amounts of  $\text{Si}_3\text{N}_4$  were added to the enamel of each wire.

One percent of  $\text{Si}_3\text{N}_4$  ceramic powder having a particle size ranging from submicron to 10 microns was added to the enamel solution of each wire (control I, control II and control III). Silicon nitride ceramic was added before the reaction of polyamideimide at the temperatures of 30° C.–90° C. The enamel was mixed with a fast-sharring device for approximately 8 hours. The resultant enamel was then passed through a filter to remove any gel particulates. The solids and viscosity of the enamel were 28%–30%, and 2000–2500 cps at 37.8° C.

The resultant enamel for each control was applied to the 18 AWG copper wires, each precoated with eight passes of polyester basecoat at the speed of 28–60 m/m in an oven having a temperature profile of 450° C.–600° C. Results were achieved with cure speeds of 28–60 m/m in an 500° C. MAG oven; and 50–60 m/m in an 600° C. MAG oven. The wall-to-wall build or thickness of the coated wire was controlled to be within 3.5 mils, and preferably within 3.0–3.3 mils. The build ratio of topcoat to basecoat was controlled to be within 15%–25% to 75%–85%. It was preferable to make 3–4 passes of the said topcoat, since a topcoat made from only 2 passes may suffer blistering or produce microbubbles. It has been found that an enamel coating built from greater than two passes is relatively insensitive to the curing conditions such as curing speed and oven temperature.

Two percent  $\text{Si}_3\text{N}_4$  ceramic powder having a particle size ranging from submicron to 10 microns was added to the enamel solution of each wire, control I, control II and control III. Silicon nitride ceramic was added before the reaction of polyamideimide at the temperatures of 30° C.–90° C. The enamel was mixed with a fast-sharring device for approximately 8 hours. The resultant enamel was then passed through a filter to remove any gel particulates. The solids and viscosity of the enamel were 28%–30%, and 2000–2500 cps at 37.8° C.

The resultant enamel for each control was also applied to the 18 AWG copper wires, each precoated with eight passes of polyester basecoat at the speed of 28–60 m/m in an oven having a temperature profile of 450° C.–600° C. The wall-to-wall build of each coated wire was controlled within 3.5 mils and preferably 3.0–3.3 mils. The build ratio of topcoat to basecoat was controlled within 15%–25% to 75%–85%.

Three percent  $\text{Si}_3\text{N}_4$  ceramic powder having a particle size ranging from submicron to 10 microns was added to the enamel solution of each wire, control I, control II and control III. Silicon nitride ceramic was added before the reaction of polyamideimide at the temperatures of 30° C.–90° C. Like the prior examples, the enamel was mixed with a fast-sharring device for approximately 8 hours. The resultant enamel was then passed through a filter to remove any gel particulates. The solids and viscosity of the enamel were 28%–30%, and 2000–2500 cps at 37.8° C.

The resultant enamel for each control was applied to the 18 AWG copper wires, each precoated with eight passes of polyester basecoat at the speed of 28–60 m/m in an oven having a temperature profile of 450° C.–600° C. The wall-to-wall build of each coated wire was controlled within 3.5 mils, and preferably within 3.0–3.3 mils. The build ratio of topcoat to basecoat was controlled within 15%–25% to 75%–85%.

Four percent  $\text{Si}_3\text{N}_4$  ceramic powder whose particle size ranges from submicron to 10 microns was added to the enamel solution of each wire, control I, control II and control III. Silicon nitride ceramic may be added before the reaction of polyamideimide at temperatures of 30° C.–90° C. The enamel was mixed with a fast-sharring device for approximately 8 hours. The resultant enamel was then passed through a filter to remove any gel particulates. The solids and viscosity of the enamel were 28%–30%, and 2000–2500 cps at 37.8° C., respectively.

The resultant enamel for each control was applied to the 18 AWG copper wires, each precoated with eight passes of polyester basecoat at the speed of 28–60 m/m in an oven having a temperature profile of 450° C.–600° C. The wall-to-wall build of each coated wire was controlled within 3.5 mils, and preferably within 3.0–3.3 mils. The build ratio of topcoat to basecoat was controlled within 15%–25% to 75%–85%.

Six percent  $\text{Si}_3\text{N}_4$  ceramic powder whose particle size ranges from submicron to 10 microns was added to the enamel solution of each wire, control I, control II and control III. Silicon nitride ceramic may be added before the reaction of polyamideimide at the temperatures of 30° C.–90° C. The enamel was mixed with a fast-sharring device for approximately 8 hours. The resultant enamel was then passed through a filter to remove any gel particles. The solids and viscosity of the enamel were 28%–30%, and 2000–2500 cps at 37.8° C.

The resultant enamel for each control was applied to the 18 AWG copper wires, each precoated with eight passes of polyester basecoat at the speed of 28–60 m/m in an oven having a temperature profile of 450° C.–600° C. The wall-to-wall build of each coated wire was controlled within 3.5 mils, and preferably within 3.0–3.3 mils. The build ratio of topcoat to basecoat was controlled within 15%–25% to 75%–85%. In an alternative embodiment, the resultant enamel was coated as a single build without the basecoat. In this embodiment the wall-to-wall build was controlled within 2.5 mils, preferably 2.0–2.3 mils.

All of these wires were prepared in an identical manner. For these wires, 9%, 12%, or 15% of  $\text{Si}_3\text{N}_4$  ceramic powder whose particle size ranges from submicron to 10 microns was added to the enamel solution of each wire, control I, control II and control III. Silicon nitride ceramic was added before the reaction of polyamideimide at the temperatures of 30° C.–90° C. The enamel was mixed with a fast-sharring device for approximately 8 hours. The resultant enamel was then passed through a filter to remove any gel particles. The solids and viscosity of the enamel were 28%–30%, and 2000–2500 cps at 37.8° C.

The resultant enamel for each control was applied to the 18 AWG copper wires, each precoated with eight passes of polyester basecoat at the speed of 28–60 m/m in an oven having a temperature profile of 450° C.–600° C. The wall-to-wall build of each coated wire was controlled within 3.5 mils, and preferably within 3.0–3.3 mils. The build ratio of topcoat to basecoat was controlled within 15%–25% to 75%–85%.

Control wires I, II and III as well as the test wires of each 60 percentage of  $\text{Si}_3\text{N}_4$  were subjected to the repeated scrape and the coefficient of friction tests. Their results are shown in the table below. For all three controls the number of repeated scrapes increased dramatically as silicon nitride was added. This indicates that silicon nitride increases the abrasion resistance of the coating. This occurred even where a minor increase in the coefficient of friction was seen. Specifically, control I shows the Rptd. S. rose from 80 with

no silicon nitride to 1010 with 6% silicon nitride by weight, and up to 1690 with a 12% increase. These increases occurred despite the fact that the C. of F. of the wire with 12% silicon nitride rose to 0.31. Adding 4% by weight silicon nitride to control II increased the Rptd. S. from 270 to 350. A 12% increase in silicon nitride increased the Rptd.S. to 1654 with C. Of F. of 0.15. Adding 3% silicon nitride to control III increased the Rptd. S. from 275 to 530 and increased to 1265 with 12% silicon nitride having a C. Of F. of 0.26. Although the data are scattered to some extent, the general trend clearly indicates a substantial increase in wire abrasion resistance as more silicon nitride is added to the wire coating.

Like the silicon nitride examples, controls I, II and III with varying amounts of AlN were subjected to the repeated scrape and the coefficient of friction. Their results are shown in the table below. For all three controls the number of 5 repeated scrapes increased dramatically as aluminum nitride was added, indicating an increase in abrasion resistance, although a minor increase in the coefficient of friction was seen. Specifically, control I shows the repeated scrape rose from 474 to 1709 with 12% AlN. AlN added to control II 10 shows an even more dramatic increase in repeated scrape. Adding just 3% AlN increases the repeated scrape from 270 to 780. Though there exists some fluctuation in the rate of repeated scrape increase, the trend still indicates a substan-

Si<sub>3</sub>N<sub>4</sub> Coated Wire  
Abrasion Resistance Comparison

|             | Amount<br>Si <sub>3</sub> N <sub>4</sub> | 0%<br>(Cntl) | 1%   | 2%   | 3%   | 4%   | 6%   | 9%  | 12%  | 15%  |
|-------------|------------------------------------------|--------------|------|------|------|------|------|-----|------|------|
| Cntl<br>I   | Build                                    | 3.2          | —    | —    | 3.4  | —    | 3.4  | —   | 3.4  | —    |
|             | Rptd.S.                                  | 80           | —    | —    | 255  | —    | 1010 | —   | 1690 | —    |
|             | C. of F.                                 | 0.28         | —    | —    | 0.24 | —    | 0.28 | —   | 0.31 | —    |
| Cntl<br>II  | Build                                    | 3.2          | 3.2  | 3.2  | 3.2  | 3.2  | 3.2  | 3.2 | 3.2  | 3.2  |
|             | Rptd.S.                                  | 270          | 290  | 340  | 280  | 350  | 350  | 513 | 1654 | 1459 |
|             | C. of F.                                 | 0.13         | 0.14 | 0.13 | 0.13 | 0.13 | 0.13 | —   | 0.15 | —    |
| Cntl<br>III | Build                                    | 3.2          | —    | —    | 3.2  | —    | 3.2  | —   | 3.2  | —    |
|             | Rptd.S.                                  | 275          | —    | —    | 430  | —    | 530  | —   | 1265 | —    |
|             | C. of F.                                 | 0.20         | —    | —    | 0.22 | —    | 0.24 | —   | 0.26 | —    |

#### Aluminum Nitride (AlN) Working Examples

In this example, varying amounts of AlN were added to each control wire. Each control wire with AlN was then tested and compared to each control wire with no AlN to determine the effects on abrasion resistance. The following illustratively describes how the varying amounts of AlN were added to the enamel of each wire.

First, 3% of AlN ceramic powder whose particle size ranges from submicron to 10 microns was added to the enamel solution of each wire, control I, control II and control III. The AlN was added after the reaction at a temperature below 120° C. because moisture in the pores degrades the formation of the polyamideimide.

The enamel was mixed with a fast-sharring device for approximately 8 hours. The resultant enamel was then passed through a filter to remove any gel particulates. The solids and viscosity of the enamel were 28%–30%, and 2000–2500 cps at 37.8° C., respectively.

The resultant enamel for each control was applied to the 18 AWG copper wires, each precoated with eight passes of polyester basecoat at the speed of 28–65 m/m in an oven having a temperature profile of 450° C.–600° C. Results were achieved with cure speeds of 28–36 m/m in an 500° C. MAG oven; and 50–60 m/m in an 600° C. MAG oven. The wall-to-wall build or thickness of the coated wire was controlled within 3.5 mils, and preferably within 3.0–3.3 mils. The build ratio of topcoat to basecoat was controlled within 15%–25% to 75%–85%. It has been demonstrated that wire coatability of this enamel is relatively insensitive to the curing condition such as curing speeds and oven temperatures. It may be preferable, however, to make 3–4 passes of the said topcoat, since the topcoat made from only 2 passes may blister or produce microbubbles. The same procedure as described above was applied to control wire I adding 6%, 9%, 12% and 15% AlN. In addition, the same procedure was applied to control wires II and III adding 3%, 6%, 9%, 12% and 15% AlN.

35  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535<br

The resultant enamel for each control was applied to the 18 AWG copper wires, each precoated with eight passes of polyester basecoat at the speed of 28–60 m/m in an oven having a temperature profile of 450° C.–600° C. Results were achieved with cure speeds of 28–36 m/m in an 500° C. MAG oven; and 50–60 m/m in an 600° C. MAG oven. The wall-to-wall build or thickness of the coated wire was controlled within 3.5 mils, and preferably within 3.0–3.3 mils. The build ratio of topcoat to basecoat was controlled within 15%–25% to 75%–85%. Generally, wire coatability of this enamel is relatively insensitive to curing such as curing speeds and oven temperatures. It may be preferable, however, to make 3–4 passes of the said topcoat, since the topcoat from only 2 passes may result in blistering or produce microbubbles. The same procedure as described above was applied to control wire I adding 2%, 3%, 4% and 10 6% TiN. In addition, the same procedure was applied to control wires II and III adding 1%, 2%, 3%, 4%, and 6% TiN.

Like the silicon nitride and aluminum nitride examples, controls I, II and III with varying amounts of TiN were subjected to the repeated scrape and the coefficient of friction. Their results are shown in the table below. For all three controls the number of repeated scrapes increased as TiN was added, indicating an increase in abrasion resistance. Specifically, though control I showed only some increase in 20 repeated scrape, control II showed a dramatic increase in repeated scrape from 270 with 0% TiN to 1520 with 6% TiN. Control III shows a similar increase in abrasion resistance. 25

| AIN Coated Wire<br>Abrasion Resistance Comparison |              |      |      |      |      |      |      |
|---------------------------------------------------|--------------|------|------|------|------|------|------|
| Amount<br>AIN                                     | 0%<br>(Cntl) | 1%   | 2%   | 3%   | 4%   | 6%   |      |
| Cntl. I                                           | Build        | 3.2  | 3.2  | 3.2  | 3.2  | 3.2  | 3.2  |
|                                                   | Rptd.S.      | 80   | 59   | 100  | 92   | 92   | 80   |
|                                                   | C. of F.     | 0.30 | 0.32 | 0.32 | 0.32 | 0.32 | 0.32 |
| Cntl. II                                          | Build        | 3.2  | 3.2  | 3.2  | 3.2  | 3.2  | 3.2  |
|                                                   | Rptd.S.      | 270  | 330  | 400  | 740  | 800  | 1520 |
|                                                   | C. of F.     | 0.14 | 0.14 | 0.14 | 0.14 | 0.14 | 0.14 |
| Cntl. III                                         | Build        | 3.2  | 3.2  | 3.2  | 3.2  | 3.2  | 3.2  |
|                                                   | Rptd.S.      | 275  | 248  | 312  | 325  | 520  | 644  |
|                                                   | C. of F.     | 0.20 | 0.22 | 0.22 | 0.23 | 0.23 | 0.23 |

I claim:

1. An abrasion resistant coated wire comprising: an electrical conductor; and a coating disposed peripherally about the electrical conductor; said coating comprising a ceramic particulate material dispersed in a polyamideimide binder; wherein the ceramic particulate material has a particle size of about 1 to 10 microns and the ceramic particulate material is present in an amount of about 1%–15% by weight of the coat.
2. The abrasion resistant coated wire of claim 1, wherein the ceramic particulate material is made from a material selected from a group consisting of silicon nitride, aluminum nitride, titanium nitride, boron nitride, molybdenum disulfide, and combinations thereof.
3. An abrasion resistant coated wire comprising: an electrical conductor having a coating disposed peripherally about the electrical conductor; and said coating comprising a ceramic particulate material and a fluoropolymer material dispersed in a polyamideimide binder; wherein the ceramic particulate material has a particle size of about 1 to 10 microns and the ceramic particu-

late material is present in an amount of about 1%–15% by weight of the coat; and wherein the fluoropolymer material is present in an amount of about 1% by weight of the coat and the fluoropolymer material has a particle size of about 0.5 to 10 microns.

4. The abrasion resistant coated wire of claim 3, wherein the ceramic particulate material is made from a material selected from a group consisting of silicon nitride, aluminum nitride, titanium nitride, boron nitride, molybdenum disulfide, and combinations thereof.

5. The abrasion resistant coated wire of claim 3, wherein the fluoropolymer is made from a material selected from a group consisting of polytetrafluoroethylene, polychlorotrifluoroethylene, polyvinylidene fluoride, fluorinated ethylene propylene, and combinations thereof.

6. An abrasion resistant coated wire comprising:

an electrical conductor; and

a coating disposed peripherally about the electrical conductor, said coating comprising a ceramic particulate material and a polyethylene material dispersed in a polyamideimide binder;

wherein the ceramic particulate material is present in an amount of about 1%–15% by weight of the coat and has a particle size of about 1 to 10 microns; and

wherein the polyethylene material has a particle size of about 5 to 15 microns and is present in an amount of about 1% by weight of the coat.

7. The abrasion resistant coated wire of claim 6, wherein the ceramic particulate material is made from a material selected from a group consisting of silicon nitride, aluminum nitride, titanium nitride, boron nitride, molybdenum disulfide, and combinations thereof.

8. An abrasion resistant coated wire comprising:

an electrical conductor;

a base insulation coat disposed peripherally about the electrical conductor; and

a top abrasion resistant coat comprising a ceramic particulate material dispersed in a polyamideimide binder; wherein the ceramic particulate material is present in an amount of about 1%–15% by weight of the coat; and wherein the ceramic particulate material has a particle size of about 1 to 10 microns.

9. The abrasion resistant coated wire of claim 8, wherein the base insulation coat is made from a material selected from a group consisting of polyester, polyesterimide, polyimide, epoxy resin, polyarylsulfone, polyether ether ketone and combinations thereof.

10. The abrasion resistant coated wire of claim 8, wherein the ceramic particulate material is made from a material selected from a group consisting of silicon nitride, aluminum nitride, titanium nitride, boron nitride, molybdenum disulfide, and combinations thereof.

11. An abrasion resistant coated wire comprising:

an electrical conductor;

a base insulation coat disposed peripherally about the electrical conductor; and

a top abrasion resistant coat comprising a ceramic particulate material and a fluoropolymer material dispersed in a polyamideimide binder;

wherein the ceramic particulate material is present in an amount of about 1%–15% by weight of the coat and has a particle size of about 1 to 10 microns; and

**11**

wherein the fluoropolymer material is present in an amount of about 1% by weight of the coat and has a particle size of about 0.5 to 10 microns.

**12.** The abrasion resistant coated wire of claim **11**, wherein the base insulation coat is made from a material selected from a group consisting of polyester, polyesterimide, polyimide, epoxy resin, polyarylsulfone, polyether ether ketone and combinations thereof. 5

**13.** The abrasion resistant coated wire of claim **11**, wherein the ceramic particulate material is made from a material selected from a group consisting of silicon nitride, aluminum nitride, titanium nitride, boron nitride, molybdenum disulfide, and combinations thereof. 10

**14.** The abrasion resistant coated wire of claim **11**, wherein the fluoropolymer is made from a material selected from a group consisting of polytetrafluoroethylene, polychlorotrifluoroethylene, polyvinylidene fluoride, fluorinated ethylene propylene, and combinations thereof. 15

**15.** An abrasion resistant coated wire comprising:  
an electrical conductor; 20  
a base insulation coat disposed peripherally about the electrical conductor; and

**12**

a top abrasion resistant coat comprising a ceramic particulate material and a polyethylene material dispersed in a polyamideimide binder;

wherein the ceramic particulate material having an amount of particulates from about 1%–15% by weight of the coat and has a particle size of about 1 to 10 microns; and

wherein the polyethylene material has a particle size of about 5 to 15 microns and is present in an amount of about 1% by weight of the coat.

**16.** The abrasion resistant coated wire of claim **15**, wherein the base insulation coat is made from a material selected from a group consisting of polyester, polyesterimide, polyimide, epoxy resin, polyarylsulfone, polyether ether ketone and combinations thereof.

**17.** The abrasion resistant coated wire of claim **15**, wherein the ceramic particulate material is made from a material selected from a group consisting of silicon nitride, aluminum nitride, titanium nitride, boron nitride, molybdenum disulfide, and combinations thereof.

\* \* \* \* \*